

1

2,802,793

## TREATMENT OF SOAP

Louis Coetzer, Rynfield, Benoni, Transvaal, Union of South Africa, and Edward Anthony Wainwright, Durban, Natal, Union of South Africa, assignors to Lever Brothers Company, New York, N. Y., a corporation of Maine

No Drawing. Application June 15, 1955,  
Serial No. 515,791

Claims priority, application Great Britain June 16, 1954

8 Claims. (Cl. 252—367)

This invention relates to the treatment of soap, particularly extruded soap of at least 20% moisture content.

It has been found that the hardness of bars or tablets (hereinafter collectively referred to as "bars") of such soap, which have been obtained by extruding the soap at a temperature not exceeding 35° C., is increased by heating them by means of alternating current to a temperature of at least 40° C. but below that at which the soap becomes no longer form-retaining due to melting and then allowing them to cool.

According to the invention there is provided a process of hardening a bar of at least 20% moisture content soap obtained by extruding the soap at a temperature not exceeding 35° C. which comprises heating the bar by means of alternating current to a temperature of at least 40° C. but below that at which the soap becomes no longer form-retaining due to melting and then allowing the bar to cool.

Preferably, the soap contains at least 25% moisture. The invention has been found particularly useful with genuine soaps having a total fatty matter content of 60-65%. The invention may also be applied to filled soaps, in particular those which contain no more than 50% moisture.

The most useful field of application of the invention is that of soap bars which have been extruded at relatively low temperatures, having regard to their moisture content, for example 25 to 30° C. in the case of genuine soaps of about 30% moisture content. The hardening effect of the process of the invention has, in general, been found most marked with those soaps which exhibit undue softening at the temperature of extrusion. Thus, for example, with genuine soaps of about 30% moisture content extruded at 25 to 30° C., the invention is most useful with soaps from fat charges containing a high percentage of low or medium titre tallow or a high percentage of rosin.

In general, the higher is the temperature to which the bar is heated the greater is the increase in hardness. It is frequently found that the rate of increase of hardness rises steeply as the melting point is approached. However, the practical difficulty of heating the soap uniformly to within a few degrees of the melting point without any substantial portion actually melting militates against working too close to this point. Also, although the lathering properties of the soaps are not usually appreciably affected by heating to temperatures in the lower portion of the range given, the increase in hardness tends to be accompanied by a sharp decrease in ease of lathering as the melting point is approached. A suitable temperature for any particular soap can easily be determined by heating samples to different temperatures, allowing them to cool, and measuring their hardness and lathering power. As a rule, temperatures within the range 45 to 55° C. have been found to be most suitable.

Once the required temperature has been reached, the soap can be allowed to cool, as there is usually little advantage to be gained by maintaining the soap at this temperature for any length of time. It is difficult to accelerate the rate of cooling of the soap. An average-size bar may take 1½ to 2 hours to cool.

2

The heating may be resistance heating by means of a low frequency alternating current, such as mains frequency current, or dielectric heating by high frequency alternating current, such as radio frequency current. The heating may be carried out batchwise by placing each bar between a pair of electrodes or continuously by passing the bar between moving endless-belt electrodes. Alternatively, the bars may be heated in the stamping dye by using opposite faces of the dye as electrodes.

5 10 The time required to reach any given temperature depends upon the nature of the soap, the thickness of the bar and, in varying degrees, depending on the mode of heating, on the potential applied, the current passing and the frequency of the current used.

15 It has been found that, as a general rule, the more rapid is the heating to the required temperature, the greater is the increase in hardness.

There may be some small loss of moisture during heating and this may tend to increase the hardness slightly but 20 the major part of the increase in hardness is not due to this cause, as can be demonstrated by carrying out the process under conditions which prevent any loss of moisture.

In the following examples, which illustrate the invention, 25 bars of soap 45.7 x 5.7 x 0.79 cm. were used. These bars were produced by rapidly chilling the molten soap, milling it, and then plodding under reduced pressure at 25 to 30° C. and cutting the plodded bar. The heating was carried out by clamping the bar of soap between two metal 30 electrodes, one at each end, with an average current of 2 amps. (the current increases as the conductivity of the soap increases with temperature) at 230 volts and 50 cycles per second. The bars took approximately 2½ to 3 minutes to reach the required temperature. Heating was 35 discontinued when the soap had reached the required temperature and the soap was then allowed to cool.

The hardness of the soaps was determined 24 hours after heating by measuring the force required to pull a wire through the soap under standardised conditions. The

40 bars were weighed before and after treatment. Control bars, that is bars not heated according to the invention, were kept in moisture-proof wrappers and their hardness measured at the same time as that of the treated bars.

### Example 1

|    |                      | Percent |
|----|----------------------|---------|
| 45 | Soap fat charge:     |         |
|    | Palm oil             | 79.5    |
|    | Olive oil            | 0.5     |
|    | Palm kernel oil      | 17.0    |
|    | Rosin                | 3.0     |
| 50 | Fatty matter content | 62.2    |

|    | Heated<br>to °C. | Hardness |        | Loss in<br>Weight<br>Percent |
|----|------------------|----------|--------|------------------------------|
|    |                  | lb.      | at °C. |                              |
| 55 |                  |          |        |                              |
|    | Control Bar      | 6.9      | 21     | 0.2                          |
|    | Hardened Bar     | 9.0      | 21     | 0.6                          |

### Example 2

|    |                      | Percent |
|----|----------------------|---------|
| 60 | Soap fat charge:     |         |
|    | Palm kernel oil      | 67      |
|    | Tallow               | 23      |
|    | Rosin                | 10      |
| 65 | Fatty matter content | 65.3    |

|    | Heated<br>to °C. | Hardness |        | Loss in<br>Weight<br>Percent |
|----|------------------|----------|--------|------------------------------|
|    |                  | lb.      | at °C. |                              |
| 70 |                  |          |        |                              |
|    | Control bar      | 4.6      | 18     |                              |
|    | Hardened Bar     | 6.6      | 18     | 0.3                          |
|    | Do.              | 6.6      | 18     | 0.3                          |

**3**  
*Example 3*

| Soap fat charge:     | Percent |
|----------------------|---------|
| Tallow (41° titre)   | 80      |
| Palm kernel oil      | 17      |
| Rosin                | 3       |
| Fatty matter content | 64.5    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 4.2      | 20     | 0.2                          |
| Hardened Bar | 49               | 5.3      | 19     | 0.4                          |
| Do           | 47               | 5.1      | 19     | 0.4                          |
| Do           | 45               | 4.9      | 19     | 0.4                          |
| Do           | 43               | 4.6      | 19     | 0.4                          |

*Example 4*

| Soap fat charge:     | Percent |
|----------------------|---------|
| Palm oil             | 80      |
| Palm kernel oil      | 17      |
| Rosin                | 3       |
| Fatty matter content | 61.5    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 7.2      | 20.5   | 0.3                          |
| Hardened Bar | 50               | 9.0      | 20     | 0.6                          |
| Do           | 40               | 8.2      | 20     | 0.6                          |

*Example 5*

| Soap fat charge:     | Percent |
|----------------------|---------|
| Coconut oil          | 80      |
| Tallow               | 20      |
| Fatty matter content | 63.0    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 6.7      | 21.5   | 0.3                          |
| Hardened Bar | 43               | 7.8      | 21.5   | 0.6                          |
| Do           | 53               | 8.5      | 21.5   | 0.6                          |

*Example 6*

| Soap fat charge:     | Percent |
|----------------------|---------|
| Palm oil             | 80      |
| Palm kernel oil      | 17      |
| Rosin                | 3       |
| Fatty matter content | 61.6    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 7.9      | 20     | 0.5                          |
| Hardened Bar | 52               | 10.7     | 20     | 0.8                          |
| Do           | 49               | 9.8      | 20     | 0.7                          |
| Do           | 46               | 9.7      | 20     | 0.7                          |
| Do           | 43               | 9.4      | 20     | 0.6                          |
| Do           | 40               | 9.4      | 20     | 0.6                          |

*Example 7*

| Soap fat charge:     | Percent |
|----------------------|---------|
| Tallow               | 63      |
| Groundnut oil        | 15      |
| Coconut oil          | 20      |
| Rosin                | 2       |
| Fatty matter content | 63.9    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 5.9      | 20     | 0.1                          |
| Hardened Bar | 52               | 7.5      | 20     | 0.3                          |
| Do           | 49               | 6.9      | 20     | 0.4                          |
| Do           | 46               | 6.7      | 20     | 0.3                          |
| Do           | 43               | 6.7      | 20     | 0.3                          |
| Do           | 40               | 6.6      | 20     | 0.3                          |

*Example 8*

| Soap fat charge:     | Percent |
|----------------------|---------|
| Palm kernel oil      | 67      |
| Tallow               | 23      |
| Rosin                | 10      |
| Fatty matter content | 62.5    |

|              | Heated<br>to °C. | Hardness |        | Loss in<br>Weight<br>Percent |
|--------------|------------------|----------|--------|------------------------------|
|              |                  | lb.      | at °C. |                              |
| Control Bar  |                  | 4.8      | 18     | 0.3                          |
| Hardened Bar | 52               | 9.7      | 18     | 0.5                          |
| Do           | 49               | 8.1      | 18     | 0.5                          |
| Do           | 46               | 6.9      | 18     | 0.4                          |
| Do           | 43               | 6.7      | 18     | 0.4                          |
| Do           | 40               | 6.7      | 18     | 0.3                          |

*Example 9*

| Soap fat charge:                 | Percent |
|----------------------------------|---------|
| Prime tallow (41.5° titre)       | 90      |
| Coconut oil                      | 10      |
| Fatty matter content             | 45.4    |
| Alkaline sodium silicate 140° Tw | 1.5     |
| Sodium carbonate                 | 0.24    |

|              | Heated<br>to °C. | Hardness |        |
|--------------|------------------|----------|--------|
|              |                  | lb.      | at °C. |
| Control Bar  |                  | 2.0      | 24.5   |
| Hardened Bar | 43.3             | 4.0      | 26.7   |
| Do           | 46.1             | 4.9      | 26.7   |
| Do           | 48.9             | 5.3      | 26.7   |
| Do           | 51.7             | 6.3      | 26.7   |
| Do           | 54.4             | 7.2      | 26.7   |

*Example 10*

| Soap fat charge:                 | Percent |
|----------------------------------|---------|
| Prime tallow (41.5° titre)       | 82      |
| Coconut oil                      | 18      |
| Fatty matter content             | 46.2    |
| Alkaline sodium silicate 140° tw | 1.5     |
| Sodium carbonate                 | 0.2     |

|              | Heated<br>to °C. | Hardness |        |
|--------------|------------------|----------|--------|
|              |                  | lb.      | at °C. |
| Control Bar  |                  | 2.3      | 22     |
| Hardened Bar | 51.0             | 7.6      | 22     |
| Do           | 48.9             | 6.5      | 22     |

*Example 11*

| Soap fat charge:           | Percent |
|----------------------------|---------|
| Prime tallow (41.8° titre) | 90      |
| Coconut oil                | 10      |
| Fatty matter content       | 45.45   |
| Neutral silicate @ 78° Tw  | 19.10   |

|              | Heated<br>to °C. | Hardness |        |
|--------------|------------------|----------|--------|
|              |                  | lb.      | at °C. |
| Control Bar  |                  | 3.3      | 25.0   |
| Hardened Bar | 48.9             | 6.9      | 26.7   |
| Do           | 54.4             | 7.8      | 26.7   |

**We claim:**

1. A process of hardening a bar of at least 20% moisture content soap obtained by extruding the soap at a temperature not exceeding 35° C., which comprises heating the bar by means of alternating current to a temperature of at least 40° C. but below that at which the soap becomes no longer form-retaining due to melting and then allowing the bar to cool.
2. A process according to claim 1 in which the soap contains at least 25% moisture.
3. A process according to claim 1 in which the soap is an unfilled soap having a total fatty matter content of 60-65%.
4. A process according to claim 1 in which the soap is a filled soap containing up to 50% moisture.
5. A process according to claim 1 in which the bar is heated by resistance heating.

6. A process according to claim 1 in which the bar is heated by dielectric heating.
7. A process according to claim 1 in which the bar is heated to a temperature in the range 45-55° C.
8. A process according to claim 3 in which the soap has been extruded at 25-30° C.

**References Cited in the file of this patent****UNITED STATES PATENTS**

10 2,527,062 Heald \_\_\_\_\_ Oct. 24, 1950

**FOREIGN PATENTS**

15 328,043 Great Britain \_\_\_\_\_ Apr. 24, 1930  
 118,453 Australia \_\_\_\_\_ Apr. 26, 1944